

Patented July 20, 1948

2,445,360

# UNITED STATES PATENT OFFICE

2,445,360

## MOTOR FUEL

Pharis Miller, Mountainside, N. J., assignor to  
Standard Oil Development Company, a corpora-  
tion of Delaware

No Drawing. Application August 31, 1946,  
Serial No. 694,437

11 Claims. (Cl. 44—69)

1

The present invention relates to an aviation fuel and more particularly relates to a fuel composition which gives improved performance in the aviation motor.

The problem of producing a proper fuel for use in the aviation motor is one that has attracted a large number of workers, due to the complexity of the requirements for a perfect fuel which will perform equally well under the different conditions encountered in the engine. For example, the fuel requirements of the aviation engine are quite different under "cruising conditions" from the conditions obtaining when the engine is accelerating during "take-off" or while the airplane is climbing.

As a solution to the problem of providing a proper aviation fuel suitable for use under the different conditions of operations, it has been proposed that aromatics, naphthenes, isoparaffins, cracked gasoline components and the like either comprise the major portion of the fuel or be added thereto in substantial amounts. Addition of tetra-ethyl lead and other anti-detonants such as amino toluenes and their homologs has also been proposed. All of these expedients, while improving the various aviation fuel base stocks, provide an improvement in the fuel's performance during either cruising conditions or during "take-off" or while the plane is climbing but not satisfying the fuel requirements suitable for both types of operation of the motor.

In accordance with the present invention, an improved aviation fuel is produced by the employment of suitable quantities of the hydrocarbon methylenecyclobutane which has the structural configuration



It is contemplated that the amount of methylenecyclobutane comprising the aviation fuel will vary with the type of base stock with which it is blended, but in general will not exceed 50% by volume of the fuel composition. It is contemplated that from 5% to 25% will be employed in most instances. It may be pointed out that methylenecyclobutane boils at a temperature in the neighborhood of 100° F. and it is desirable for the complete blend to have a Reid pressure in the neighborhood of 7 pounds per square inch at 100° F. This limitation of vapor pressure is de-

2

signed to prevent vapor lock and excessive evaporation of the fuel.

The methylenecyclobutane may be employed in a fuel composition, the other constituents of which are predominantly isoparaffinic in nature. Thus, besides methylenecyclobutane, the fuel may comprise isopentane, isohexane, isoheptane, iso-octane and the like. The improved fuel of my invention may also include amounts of tetraethyl lead, iron carbonyl and other anti-detonants such as the class of compounds illustrated by the amino toluenes.

In some instances it may be desirable to prepare a fuel in accordance with the present invention which comprises methylenecyclobutane and quantities of the aromatics and/or naphthenes. Mixtures of the latter types of hydrocarbons with isoparaffins form suitable base stocks to which the methylenecyclobutane may be added.

15 The isoparaffins may be obtained from naturally occurring sources or may be produced synthetically as by the well known alkylation and/or isomerization reactions. Irrespective of the source of the isoparaffins, it is preferred to employ them in my fuel composition in relatively pure form.

20 Suitable fractions of crude petroleum from crude oils of the Coastal type, which boil in the gasoline boiling range, may also form the base stock of my improved fuel. Generally, the hydrocarbon fractions will not have a boiling point which exceeds 350° F. When using crude petroleum fractions with methylenecyclobutane, it may be desirable to employ other blending agents such as alkylates and tetraethyl lead to obtain maximum utilization of the qualities of the admixture. The tetraethyl lead may be employed in most instances, in amounts not exceeding 6 cc. per gallon of fuel.

25 30 35 40 The compound methylenecyclobutane has been described in the literature (see for example Berichte der deutschen chemischen Gesellschaft v. 72:2021-2026 (1939) and Journal American Chemical Society v. 64:1142-7 (1942)).

45 It is suitably prepared from pentaerythritol bromide as follows: 100 g. of pentaerythritol bromide and 250 g. of zinc powder were placed in a reaction flask and 250 cc. of 50% ethyl alcohol was slowly added. A hot water bath was placed around the flask until a localized reaction started. The product distilling over at 38° to 41° C. (100.4°-105.8° F.) was washed and dried over calcium chloride and identified as methylenecyclobutane. It was tested by the A. S. T. M.

motor method and found to have a blending octane number of 99.

As a specific example of the improved fuel composition, an aviation fuel in accordance with the present invention may be prepared by adding 20 parts of methylenecyclobutane to 80 parts of an alkylate having a vapor pressure of four pounds Reid. The vapor pressure of this composition is slightly over 6 pounds Reid and is satisfactory for use in an aviation motor.

In another example, a fuel, in accordance with the present invention, is prepared by blending 25 parts of methylene-cyclobutane with a mixture composed of equal parts of 2, 2-dimethyl-butane, commonly called neo-hexane and iso-octane. This 15 composition is also satisfactory for use as an aviation fuel.

The nature and objects of the present invention having been described and illustrated, what is claimed as new and useful and desired to be secured by Letters Patent is:

1. An aviation fuel consisting essentially of a minor portion of methylenecyclobutane and a major portion of hydrocarbons boiling in the gasoline boiling range.
2. An aviation fuel in accordance with claim 1 in which the hydrocarbons boiling in the gasoline boiling range are obtained from crude petroleum.
3. An aviation fuel in accordance with claim 1 in which the hydrocarbons boiling in the gasoline range are produced synthetically.
4. An aviation fuel in accordance with claim 1 in which the methylenecyclobutane comprises less than 50% by volume of the fuel.
5. An aviation fuel consisting essentially of a minor amount of methylenecyclobutane and a

major amount of isoparaffinic hydrocarbons boiling in the gasoline boiling range.

6. An aviation fuel in accordance with claim 5 in which the minor amount of methylenecyclobutane comprises less than 50% by volume of the fuel.

7. An aviation fuel in accordance with claim 1 which comprises tetraethyl lead.

8. An aviation fuel in accordance with claim 5 which comprises tetraethyl lead.

9. An aviation fuel consisting essentially of methylenecyclobutane as a minor component and a mixture of isoparaffinic, naphthenic and aromatic hydrocarbons boiling in the gasoline boiling range as a major component.

10. An aviation fuel in accordance with claim 9 which comprises tetraethyl lead.

11. An aviation fuel containing anti-detonants consisting essentially of a minor portion of methylenecyclobutane and a major portion of hydrocarbons boiling in the gasoline boiling range.

PHARIS MILLER.

#### REFERENCES CITED

The following references are of record in the file of this patent:

#### UNITED STATES PATENTS

| 30 | Number    | Name      | Date           |
|----|-----------|-----------|----------------|
|    | 2,407,717 | Marschner | Sept. 17, 1946 |
|    | 2,411,582 | McCulloch | Nov. 26, 1946  |

#### OTHER REFERENCES

|    |                                                                                                     |
|----|-----------------------------------------------------------------------------------------------------|
| 35 | Slabey, National Advisory Committee for Aeronautics, Technical Note 1023, February 1946, pages 1-9. |
|----|-----------------------------------------------------------------------------------------------------|